

# UNITED STATES PATENT OFFICE.

HARTLEY FLETCHER, OF THAON-LES-VOSGES, FRANCE, ASSIGNOR TO ALPHONSE  
EMILE VERGÉ, OF VINCENNES, FRANCE.

## DYEING OF FABRICS AND FIBERS WITH ANILIN-BLACK BY OXIDATION IN THE AIR.

1,119,075.

Specification of Letters Patent.

Patented Dec. 1, 1914.

No Drawing.

Application filed August 20, 1913. Serial No. 785,769.

To all whom it may concern:

Be it known that I, HARTLEY FLETCHER, a subject of the King of Great Britain, and resident of Thaon-les-Vosges, France, have invented new and useful Improvements in the Dyeing of Fabrics and Fibers with Anilin-Black by Oxidization in the Air, which are fully set forth in the following specification.

10 The present invention relates to anilin black dyeing, and more particularly to anilin dyeing as practised according to the process disclosed in my prior Letters Patent, Number 1,102,898, granted July 7, 1914.

15 The chief feature of the patented process is the subjection of the fabrics or fibers to the action of a dye bath which consists of anilin, paraphenylenediamin, hydrochloric acid, formic acid, copper-sulfate and sodium bisulfite in certain specified proportions, as may be ascertained from said patent, the material to be dyed, after having been treated with such bath, being successively dried and subjected to a finishing treatment.

25 It is the object of this invention to improve the patented bath by reducing the quantity of the paraphenylenediamin and its solvent, formic acid, and of the sodium bisulfite, and by increasing the quantity of the copper-salts, as a result of which, a fast black may be obtained without requiring any finishing treatment of the material, although such treatment may, if desired, be carried out, in order to render the color absolutely incapable of turning green, and to insure all portions of the material being sufficiently oxidized.

According to the present invention, the improved dye bath is composed of the following ingredients in substantially the proportions stated, viz:—

|                           |           |
|---------------------------|-----------|
| Anilin                    | 45 grams. |
| Paraphenylenediamin       | 3 grams.  |
| Hydrochloric acid         | 35 grams. |
| 90% formic acid           | 5 grams.  |
| Copper sulfate            | 9 grams.  |
| Copper acetate            | 3 grams.  |
| Dry sodium bisulfite      | 2 grams.  |
| Water to make up 1 liter. |           |

As will be seen from a comparison of the above formula with that disclosed in the patent, to which latter reference may be had for a complete understanding of the process, the present bath contains 3 grams less of

paraphenylenediamin, 5 grams less of formic acid, and 1 gram less of sodium bisulfite, but contains 3 grams more of copper sulfate, and, in addition, 3 grams of copper acetate, which has no counterpart in the earlier bath. However, the quantity of paraphenylenediamin contained in the present bath still greatly exceeds that included in the ordinary anilin black dye bath, while the quantity of copper salts of the present bath still is greatly less than that in the ordinary bath. Moreover, if desired, the copper sulfate in the present bath may be either wholly or partly replaced by copper acetate, with advantageous results, especially if a finishing treatment is to be employed since the danger of the material being weakened during such treatment is greatly reduced.

In carrying out the present process, the material undergoing treatment, after having been impregnated by repeated immersions in the bath, is dried in any suitable manner, as, for instance, by being suspended in a drying room for 48 hours, or left in a heap for the same period of time, during which period they are repeatedly aerated, to produce oxidation in the air. Excellent results are even obtained by causing the material to oxidize in the air for only 24 hours, and even for 12 hours.

As previously stated, the employment of the improved bath renders a finishing treatment unnecessary, although such treatment may be followed when it is desired to completely avoid all danger of the color turning, and to insure complete oxidation. When this step is made use of, it is deemed preferable to carry it out after chromation, the material being passed through a bath composed of anilin oil, or its homologues or analogues, instead of through a bath composed of an anilin salt dissolved in water, or its homologues, as in the patented process. The proportion of anilin oil may extend, if desired, to saturation.

I claim:—

1. The herein-described bath for dyeing textile material which consists of 45 grams of anilin, 3 grams of paraphenylenediamin, 35 grams of hydrochloric acid, 5 grams of 90% formic acid, 12 grams of copper salts, 2 grams of dry sodium bisulfite, and water to make up 1 liter.

2. The herein-described bath for dyeing textile material which consists of 45 grams

of anilin, 3 grams of paraphenylenediamin,  
35 grams of hydrochloric acid, 5 grams of  
90% formic acid, 12 grams of copper salts,  
including copper acetate, 2 grams of dry  
5 sodium bisulfite, and water to make up 1  
liter.

In testimony whereof I have signed this

specification in the presence of two subscrib-  
ing witnesses.

HARTLEY FLETCHER.

Witnesses:

EMILE LEDRET,  
HANSON C. COXE.